# EUROPEAN PATENT SPECIFICATION

(11) **EP 2 103 697 B1**
(45) Date of publication and mention of the grant of the patent: **01.05.2019**
(21) Application number: 07860538.3
(22) Date of filing: 21.12.2007
(51) Int. Cl.: C22C 38/00, C22C 38/02, C22C 38/04, C22C 38/06, C22C 38/08, C22C 38/38, C21D 9/46, C21D 8/02

(54) **HIGH CARBON HOT-ROLLED STEEL SHEET**
KOHLENSTOFFREICHES HEISSGEWALZTES STAHLBLECH
TÔLE EN ACIER LAMINÉ À CHAUD À TENEUR EN CARBONE ÉLEVÉE

(30) Priority: 25.12.2006 JP 2006347539
(43) Date of publication of application: 23.09.2009
(73) Proprietor: JFE Steel Corporation, Tokyo 100-0011 (JP)
(72) Inventor: KARIYA, Nobusuke, Tokyo 100-0011 (JP); SETO, Kazuhiro, Tokyo 100-0011 (JP); NAKAMURA, Nobuyuki, Tokyo 100-0011 (JP)
(74) Representative: Grünecker Patent- und Rechtsanwälte PartG mbB
(86) International application number: PCT/JP2007/075341
(87) International publication number: WO 2008/081956

(56) References cited:
- EP-A1- 1 980 635
- EP-A1- 2 003 220
- JP-A- H0 987 798
- JP-A- S5 550 427
- JP-A- 04 214 839
- JP-A- 05 239 588
- JP-A- 10 265 845
- JP-A- 55 050 427
- JP-A- 62 284 019
- JP-A- H10 265 845
- JP-A- S62 284 019
- JP-A- 2001 214 234
- JP-A- 2003 013 145
- JP-A- 2005 097 740
- JP-A- 2005 290 547
- JP-A- 2006 063 394
- JP-A- 2007 039 796
- JP-A- 2007 277 696

## Description

### Technical Field

The present invention relates to a high-carbon hot-rolled steel sheet, particularly a high-carbon hot-rolled steel sheet having excellent bending properties after processing, and a method of producing the same.

### Background Art

High-carbon steel sheets used for tools or automobile parts (gear and transmission) are required by users to have excellent workability because they are worked into various complex shapes. On the other hand, in recent years, reduction in manufacturing cost of parts has been strongly required, resulting in the omission of a working process and a change in a working method. For example, as described in Non-Patent Document 1, a double-acting forming technique which permits thickness-additive forming process and realizes a significant reduction in the process is disclosed as a processing technique for automobile driving-system parts using high-carbon steel sheets and partially put into practical application. Accordingly, high-carbon steel sheets are required to be processable without a problem even when a plurality of processing types such as stretching, drawing, bulging, bending, and hole-expansion (burring) are combined. In particular, when bending is performed after tension, a crack frequently occurs in a bent portion, and thus excellent bending properties after stretching are required.

In order to improve workability of high-carbon steel sheets, several techniques have been investigated so far. For example, Patent Document 1 proposes a method in which high-carbon steel having predetermined chemical components is hot-rolled, descaled, annealed in an atmosphere containing 95% by volume or more of hydrogen at a heating rate for a soaking time which are specified according to the chemical components, and then cooled at a cooling rate of 100 °C/hr or less to produce a high-carbon workable steel strip having a uniform microstructure and excellent workability. Patent Document 2 proposes a method in which a steel sheet rolled at a finishing temperature of (Ac₁ transformation point + 30°C) or more is cooled to a temperature of 20 to 500°C at a cooling rate of 10 to 100 °C/sec, maintained for 1 to 10 seconds, reheated in a temperature range of 500°C to (Ac₁ transformation point + 30°C), and then coiled, and, if required, soaked at 650°C to (Ac₁ transformation point + 30°C) for 1 hour or more to produce a high-carbon thin steel sheet having good workability. Further, Patent Document 3 proposes a method in which steel containing 0.2 to 0.7% by mass of C is hot-rolled at a finishing temperature of (Ar₃ transformation point - 20°C) or more, cooled at a cooling rate of over 120 °C/sec and a cooling stop temperature of 650°C or less, coiled at a coiling temperature of 600°C or less, and then annealed at an annealing temperature of 640°C to Ac₁ transformation point to produce a high-carbon hot-rolled steel sheet having excellent stretch-flangeformability.

Non-patent Document 1: Journal of the JSTP, 44, 2003, p. 409-413
Patent Document 1: Japanese Unexamined Patent Application Publication No. 9-157758
Patent Document 2: Japanese Unexamined Patent Application Publication No. 5-9588
Patent Document 1: Japanese Unexamined Patent Application Publication No. 2003-13145

Other previously proposed arrangements are disclosed in document JP S55 50427 A.

### Disclosure of Invention

However, the high-carbon hot-rolled steel sheets described in these conventional techniques have excellent properties when processed by a single processing type such as stretching or hole-expansion, but has the problem of producing cracks when bending is performed after stretching, i.e., when a plurality of processing types are combined.

The present invention provides a high-carbon hot-rolled steel sheet having excellent bending properties after stretching and a method of producing the same.

As a result of intensive research on the bending properties of a high-carbon hot-rolled steel sheet after stretching, the inventors have found that it is very important to appropriately control a Sol. Al content in steel, cooling conditions after hot rolling, a coiling temperature, and an annealing temperature. Also the inventors have found that when a ferrite grain diameter measured by a measurement method, which will be described below, is controlled to 5.0 µm or less, and the area ratio of ferrite grains with an aspect ratio of 4.0 or more is controlled to 15% or less, excellent bending properties after stretching are achieved.

The present invention has been achieved on the basis of the above-mentioned findings and provides a high-carbon hot-rolled steel sheet which is a hot-rolled spheroidizing annealed material, the steel sheet having a composition consisting of, in % by mass, 0.2 to 0.7% of C, 2% or less of Si, 2% or less of Mn, 0.03% or less of P, 0.03% or less of S, 0.01% or less of Sol. Al, and 0.01% or less of N, optionally at least one selected from B, Cr, Ni, Mo, Cu, Ti, Nb, W, V, and Zr in the following content ranges in % by mass: B: 0.005% or less, Cr: 3.5% or less, Ni: 3.5% or less, Mo: 0.7% or less, Cu: 0.1% or less, Ti: 0.1% or less, Nb: 0.1% or less, W, V, Zr: 0.1% or less in total, the balance being Fe and inevitable impurities, a ferrite grain diameter being 5.0 µm or less, and an area ratio of ferrite grains with an aspect ratio of 4.0 or more being 15% or less.

The ferrite grain diameter is an average grain diameter determined by approximating ferrite grains as circular grains in image analysis, and the aspect ratio is an average value of (major axis of ellipse)/(minor axis of ellipse) determined by approximating ferrite grains as elliptic grains in image analysis. Specifically, a section of the steel sheet in a direction parallel to the rolling direction is polished and etched a nital solution (nitric acid + ethanol) at a position of 1/4 thickness of the sheet, and then a microstructure is observed with a scanning electron microscope at a magnification of 1500× to determine a ferrite grain diameter and the aspect ratio of a ferrite grain by image analysis using an image analysis software "Image Pro Plus ver. 4.0" (TM) manufactured by Media Cybernetics Co., Ltd. The area ratio of ferrite grains with an aspect ratio of 4.0 or more is determined and then divided by the total area of the field of view to determine the area ratio of each field of view. The average of 50 fields of view is regarded as the area ratio of ferrite grains with an aspect ratio of 4.0 or more.

The area ratio of the ferrite grains with an aspect ratio of 4.0 or more is preferably 10% or less.

According to the present invention, a high-carbon hot-rolled steel sheet exhibiting excellent bending properties even after processing such as stretching can be produced.

### Brief Description of Drawings

Fig. 1 is a graph showing a relation between the area ratio of ferrite grains with an aspect ratio of 4.0 or more and bending properties after stretching.

### Best Mode for Carrying Out the Invention

A high-carbon hot-rolled steel sheet and a method of producing the same according to the present invention will be described in detail below. The unit "%" of the content of each component represents "% by mass" unless otherwise specified.

### Composition of steel

C content: C is an important element which forms a carbide and provides hardness after quenching. When the C content is less than 0.2%, sufficient strength as machine structural parts cannot be obtained after quenching. On the other hand, when the C content exceeds 0.7%, a sufficient bending property after stretching cannot be obtained even when the ferrite grain diameter is 5.0 µm or less and the area ratio of ferrite grains with an aspect ratio is 15% or less. Also, the hardness after hot rolling is significantly increased, and the steel sheet becomes brittle to cause disadvantage in handling and saturate strength as machine structural parts after quenching. Therefore, the C content is specified to 0.2 to 0.7%. When hardness after quenching is regarded as more important, the C content preferably exceeds 0.5%, while when workability is regarded as important, the C content is preferably 0.5% or less.

Si content: Si graphitizes a carbide and tends to inhibit hardenability, and thus the content is 2% or less and preferably 1% or less.

Mn content: When Mn is excessively contained, ductility tends to be decreased. Therefore, the Mn content is specified to 2% or less and preferably 1% or less.

P content: When P is excessively contained, ductility such as stretch-flange properties is decreased, and cracks easily occur. Therefore, the P content is 0.03% or less and preferably 0.02% or less.

S content: When S is excessively contained, ductility such as stretch-flangeformability is decreased, and cracks easily occur. Therefore, the S content is 0.03% or less and preferably 0.07% or less.

Sol. Al content: Sol. Al is the most important element in the present invention. Namely, the inventors newly found that when the Sol. Al content exceeds 0.01%, AlN is formed on a surface layer of the steel sheet in annealing the hot-rolled steel sheet in a nitrogen atmosphere using nitrogen which is relatively inexpensive and frequently used as a non-oxidizing atmosphere, and the surface layer of the steel sheet is hardened to significantly decrease the bending properties after stretching. Therefore, the Sol. Al content is specified to 0.01% or less.

N content: When N is excessively contained, ductility is decreased. Therefore, the N content is 0.01% or less and preferably 0.005% or less.

Since the cost is increased by decreasing the content of each of the above elements to a predetermined amount, for example, less than 0.0001%, the content of each element is preferably about 0.0001% or more.

The balance is composed of Fe and inevitable impurities, but even when at least one element of B, Cr, Ni, Mo, Cu, Ti, Nb, W, V, and Zr may be added in a usual range in order to improve hardenability by quenching and resistance to temper softening, the advantage of the present invention is not impaired.

Specifically, these elements can be contained at the following contents: B: 0.005% by or less, Cr: 3.5% or less, Ni: 3.5% or less, Mo: 0.7% or less, Cu: 0.1% or less, Ti: 0.1% or less, Nb: 0.1% or less, W, V, Zr: 0.1% or less in total. For this purpose, the elements are preferably contained at the following contents: B: 0.0005% or more, Cr: 0.05% or more, Ni: 0.05% or more, Mo: 0.05% or more, Cu: 0.01% or more, Ti: 0.01% or more, Nb: 0.01% or more, W, V, Zr: 0.01% or more in total. Further, even when elements such as Sn, Pb, and the like are mixed as impurities in the production process, the advantage of the present invention is not affected.

### Production condition

Finishing temperature of hot rolling: When the finishing temperature is lower than (Ar₃ transformation point - 20°C), the steel sheet is partially rolled in a ferrite transformation region, and thus the ferrite grain diameter after annealing exceeds 5.0 µm, thereby degrading the bending properties after stretching. Therefore, the finishing temperature of hot rolling is (Ar₃ transformation point - 20°C) or more. Although the Ar₃ transformation point can be calculated from the equation (1) below, an actually measured temperature may be used. ${Ar}_{3} transformation point = 910 - 203 \times {\left[C\right]}^{1 / 2} + 44.7 \times \left[Si\right] - 30 \times \left[Mn\right]$ wherein [M] represents the content (%) of element M. Further, correction terms may be introduced according the elements contained. For example, when Cr, Mo, and Ni are contained, the correction terms, such as - 11 × [Cr], + 31.5 × [Mo], and - 15.2 × [Ni], may be added to the right side of the equation (1).

Cooling condition after hot rolling: In the present invention, grain refining of ferrite grains is achieved in spite of the low Sol. Al content and difficulty in inhibiting grain growth by AlN pinning. This is estimated to be due to the fact that strain applied to austenite grains during rolling is easily accumulated by rapid cooling after hot rolling, and the accumulated strain contributes as nucleation sites of ferrite grains during subsequent annealing. When the cooling rate after hot rolling is less than 60 °C/sec, the strain applied to the austenite grains during rolling is little accumulated, and thus the number of the nucleation sites of ferrite grains is decreased in subsequent annealing, thereby accelerate the growth of ferrite grains. As a result, the ferrite grain diameter exceeds 5.0 µm, and the bending properties after stretching are degraded. On the other hand, when the cooling rate is 120 °C/sec or more, the ferrite grain diameter after annealing is 5.0 µm or less, but the area ratio of ferrite grains with an aspect ratio of 4.0 or more exceeds 15%. Therefore, as described above, the bending properties after stretching are degraded. This is estimated to be due to the fact that when the cooling rate is 120 °C/sec or more, the strain applied to the austenite grains during rolling is excessively present after rolling, thereby causing difficulty in growth of equiaxial ferrite grains in subsequent annealing. Therefore, the cooling rate after hot rolling is 60 °C/sec to less than 120 °C/sec. The upper limit of the cooling rate is preferably 115 °C/sec.

When the end-point of cooling of the hot-rolled steel sheet at the above-described cooling rate, i.e., the cooling stop temperature, is higher than 650°C, the strain accumulated in austenite in cooling is released until the hot-rolled steel sheet is coiled. As a result, the ferrite grain diameter after annealing exceeds 5.0 µm, and thus the bending properties after stretching are degraded. Therefore, the cooling stop temperature is 650°C or less and preferably 600°C or less. In view of the problem with measurement accuracy of the temperature, the cooling stop temperature is preferably 500°C or more.

Cooling after the cooling stop temperature is attained is not particularly specified, and natural cooling or accelerated cooling with deceased cooling force may be continued. From the viewpoint of homogeneous mechanical properties of the steel sheet, accelerated cooling is preferably performed to an extent which suppresses regeneration of heat.

Coiling temperature: The hot-rolled steel sheet after cooling is coiled. When the coiling temperature exceeds 600°C, the strain accumulated in austenite during hot rolling is released. As a result, the ferrite grain diameter after annealing exceeds 5.0 µm, and thus the bending properties after stretching are degraded. Therefore, the coiling temperature is 600°C or less. In order to obtain the sufficient effect of cooling, the coiling stop is preferably lower than the cooling termination temperature. Since the shape of the hot-rolled steel sheet is degraded, the coiling temperature is preferably 200°C or more and more preferably 350°C or more.

When the area ratio of ferrite grains with an aspect ratio of 4.0 or more is 10% or less, the bending properties are further improved. In this case, it is necessary that the cooling rate is 80 °C/sec to less than 120 °C/sec, the cooling stop temperature is 600°C or less, and the coiling temperature is 550°C or less.

Descaling: The hot-rolled steel sheet after coiling is generally descaled before subsequent annealing. The descaling means is not particularly limited, but pickling by a usual method is preferred.

Annealing temperature of hot-rolled steel sheet: After descaling by pickling, the hot-rolled steel sheet is annealed by spheroidizing annealing for spheroidizing carbides. When the annealing temperature is less than 640°C, growth of ferrite grains is insufficient, and thus the area ratio of ferrite grains with an aspect ratio of 4.0 or more exceeds 15%, thereby deteriorating the bending properties after stretching. On the other hand, when the annealing temperature exceeds the Ac₁ transformation point, austenite formation partially proceeds to form pearlite during cooling, thereby deteriorating the bending properties after stretching. Therefore, the annealing temperature of the hot-rolled steel sheet is 640°C to the Ac₁ transformation point. In order to obtain more excellent stretch-flangeability, the annealing temperature of the hot-rolled steel sheet is preferably 680°C or above. Although the Ac₁ transformation point can be calculated from the equation (2) below, an actually measured temperature may be used. ${Ac}_{1} transformation point = 754.83 - 32.85 \times \left[C\right] + 23.32 \times \left[Si\right] - 17.76 \times \left[Mn\right]$ wherein [M] represents the content (%) of element M. Further, correction terms may be introduced according the elements contained. For example, when Cr, Mo, and V are contained, the correction terms, such as + 17.3 × [Cr], + 4.51 × [Mo], and + 15.62 × [V], may be added to the right side of the equation (2).

The annealing time of the hot-rolled steel sheet is preferably about 8 to 80 hours. The carbide in the resultant steel sheet is spheroidized, and the average aspect ratio is about 5.0 or less (a value measured at a position of about 1/4 thickness of the sheet).

For steel making of the high-carbon steel according to the present invention either a converter or an electric furnace can be applied. Thus made high-carbon steel is formed into a slab by ingoting and blooming or continuous casting. The slab is generally heated, (reheated), and then treated by hot-rolled.

For the slab manufactured by continuous casting may be treated by hot direct rolling directly from the slab or after heat-holding to prevent temperature reduction. For the case of hot-rolling the slab after reheating, the slab heating temperature is preferably specified to 1280°C or below to avoid the deterioration of surface condition caused by scale.

The hot-rolling can be given only by finishing rolling eliminating rough rolling. To assure the finishing temperature, the material being rolled may be heated during hot-rolling using a heating means such as sheet bar heater. To enhance spheroidization or to decrease hardness, the coiled sheet may be thermally insulated by a slow-cooling cover or other means.

Although the thickness of the hot-rolled sheet is not specifically limited if only the manufacturing conditions of the present invention are maintained, a particularly preferable range of the thickness thereof is from 1.0 to 10.0 mm from the point of operability.

The annealing of hot-rolled sheet can be done either by box annealing or by continuous annealing. After annealing or hot-rolled sheet, skin-pass rolling is applied, at need. Since the skin-pass rolling does not affect the hardenability by quenching, there is no specific limitation or the condition of skin-pass rolling.

The hot-rolled steel sheet produced by the above-described method of the present invention is a hot-rolled steel sheet subjected to hot-rolling spheroidizing annealing and containing carbides spheroidized to an average aspect ratio of about 5.0 or less.

The hot-rolled steel sheet of the present invention has a ferrite grain diameter of 5.0 µm or less. The ferrite grain diameter affects the bending properties after stretching. When the ferrite grain diameter exceeds 5.0 µm, many fine carbide grains are precipitated in ferrite grains, and voids produced by stretching at interfaces between carbides and ferrite are connected together during bending to cause cracks. When the ferrite grain diameter is 5.0 µm or less, the number of carbide in ferrite grains is decreased, and the fine voids produced by stretching are little connected by bending after stretching, thereby suppressing the occurrence of cracks.

Further, in the hot-rolled steel sheet of the present invention, the area ratio of ferrite grains with an aspect ratio of 4.0 or more is 15% or less. Like the ferrite grain diameter, the shape of ferrite grains affects the bending properties after stretching. When the aspect ratio of the ferrite grains is 4.0 or more, fine cracks easily occur by stretching at grain boundaries between ferrite grains with an aspect ratio of 4.0 or more and equiaxial ferrite grains with an aspect ratio less than 4.0. When the area ratio of such ferrite grains with an aspect ratio of 4.0 or more exceeds 15%, cracking starts in bending at fine cracks produced in stretching. When the area ratio of ferrite grains with an aspect ratio of 4.0 or more is 15% or less, the occurrence of cracks in bending after stretching can be suppressed. The area ratio of ferrite grains with an aspect ratio of 4.0 or more is more preferably 10% or less.

### EXAMPLE 1

Continuously cast slabs of steels A to E and Z having the chemical compositions shown in Table 1 were heated to 1250°C, hot-rolled under the conditions shown in Table 2, pickled, and then annealed under the conditions shown in Table 2 to produce steel sheet Nos. 1 to 20 having a thickness of 5. 0 mm. Annealing was performed in a nitriding atmosphere (N₂ atmosphere).

Steel sheets Nos. 1 to 10 are examples of the present invention, and steel sheet Nos. 11 to 20 are comparative examples. The ferrite grain diameter and the aspect ratio and area ratio of ferrite grains were measured by the following methods. The bending properties after stretching were also measured by the following method.

Ferrite grain diameter and aspect ratio and area ratio of ferrite grains: The ferrite grain diameter is an average grain diameter determined by approximating ferrite grains as circular grains in image analysis, and the aspect ratio is an average value of (major axis of ellipse)/(minor axis of ellipse) determined by approximating ferrite grains as elliptic grains in image analysis. Specifically, a thickness section of the steel sheet in a direction parallel to the rolling direction was polished and etched a nital solution (nitric acid + ethanol) at a position of 1/4 thickness of the sheet, and then a microstructure was observed with a scanning electron microscope at a magnification of 1500× to determine a ferrite grain diameter and the aspect ratio of a ferrite grain by image analysis using an image analysis software "Image Pro Plus ver. 4.0" (TM) manufactured by Media Cybernetics Co., Ltd. The area ratio of ferrite grains with an aspect ratio of 4.0 or more was determined and then divided by the total area of a field of view to determine the area ratio of each field of view. The average of 50 fields of view was regarded as the area ratio of ferrite grains with an aspect ratio of 4.0 or more.

Further, a thickness section of the steel sheet in a direction parallel to the rolling direction was polished and etched a picral solution (picric acid + ethanol) at a position of 1/4 thickness of the sheet, and then a microstructure was observed with a scanning electron microscope at a magnification of 3000× to determine the aspect ratio (maximum diameter)/(minimum diameter) of carbide using the image analysis software. The aspect ratios of carbides were averaged (number average) to determine the average aspect ratio. As a result, it was confirmed that the carbides were spheroidized and annealed.

Bending properties after stretching: A tensile test was performed by a method according to JIS Z 2241 using a JIS No. 5 test piece obtained in a direction perpendicular to the rolling direction and having a parallel portion of 30 mm in width to apply predistortion of 15%, and then a bending test was performed by a pressing bend method according to JIS Z 2249. The bending test was performed three times using a punch diameter D of 1 mm. When no crack occurred in the three tests, the bending property was decided as ○, when cracks occurred one time or two times, the bending property was decided as Δ, and when cracks occurred three times, the bending property was decided as ×. In the case of ○, the test piece was considered as an example of the present invention.

The results are shown in Table 3. In steel sheet Nos. 1 to 10 as examples of the present invention, the ferrite grain diameter is 5.0 µm or less, the area ratio of ferrite grains with an aspect ratio of 4.0 or more is 15% or less, and thus the bending property after stretching is excellent. In each of the examples of the present invention, it was confirmed that the average aspect ratio of carbides is 5.0 or less, and the carbides are spheroidized by spheroidizing annealing.

Fig. 1 shows a relation between the area ratio of ferrite grains with an aspect ratio of 4.0 or more and bending property after stretching when the ferrite grain diameter is 5.0 µm or less. As in steel sheet Nos. 1 to 10 as the examples of the present invention, when the ferrite grain diameter is 5.0 µm or less, and the area ratio of ferrite grains with an aspect ratio of 4.0 or more is 15% or less, the excellent bending property after stretching can be obtained.

**Table 1**

| (% by mass) | | | | | | | | | |
|---|---|---|---|---|---|---|---|---|---|
| Steel | C | Si | Mn | P | S | Sol. Al | N | Ar₃ transformation point determined from equation (1) | Ac₁ transformation point determined from equation (2) |
| A | 0.26 | 0.22 | 0.83 | 0.010 | 0.0025 | 0.007 | 0.0031 | 791 | 737 |
| B | 0.34 | 0.20 | 0.74 | 0.015 | 0.0018 | 0.005 | 0.0033 | 778 | 735 |
| C | 0.35 | 0.02 | 0.15 | 0.009 | 0.0030 | 0.006 | 0.0036 | 786 | 741 |
| D | 0.49 | 0.19 | 0.76 | 0.011 | 0.0027 | 0.010 | 0.0032 | 754 | 730 |
| E | 0.66 | 0.21 | 0.75 | 0.014 | 0.0045 | 0.003 | 0.0030 | 732 | 725 |
| Z | 0.36 | 0.21 | 0.73 | 0.013 | 0.0022 | 0.032 | 0.0032 | 776 | 735 |

**Table 2**

| Steel sheet No. | Steel | Hot rolling condition | | | | Annealing of hot-rolled steel sheet | Remarks |
|---|---|---|---|---|---|---|---|
| | | Finishing temperature (°C) | Cooling rate (°C/sec) | Cooling stop temperature (°C) | Coiling temperature (°C) | | |
| 1 | A | 801 | 110 | 620 | 550 | 700°C×40hr | Example of this invention |
| 2 | A | 811 | 95 | 560 | 510 | 720°C×40hr | Example of this invention |
| 3 | B | 788 | 115 | 610 | 540 | 680°C×40hr | Example of this invention |
| 4 | B | 808 | 85 | 570 | 520 | 710°C×40hr | Example of this invention |
| 5 | C | 801 | 75 | 610 | 590 | 670°C×40hr | Example of this invention |
| 6 | C | 806 | 105 | 580 | 490 | 720°C×40hr | Example of this invention |
| 7 | D | 774 | 90 | 620 | 580 | 710°C×40hr | Example of this invention |
| 8 | D | 784 | 100 | 550 | 500 | 720°C×40hr | Example of this invention |
| 9 | E | 752 | 65 | 600 | 570 | 700°C×40hr | Example of this invention |
| 10 | E | 772 | 100 | 540 | 490 | 720°Cx40hr | Example of this invention |
| 11 | A | 801 | 80 | 680 | 580 | 700°C×40hr | Comp. Example |
| 12 | A | 751 | 100 | 610 | 570 | 700°C×40hr | Comp. Example |
| 13 | B | 798 | 110 | 620 | 560 | 600°C×40hr | Comp. Example |
| 14 | B | 793 | 90 | 600 | 630 | 690°C×40hr | Comp. Example |
| 15 | C | 816 | 150 | 580 | 520 | 720°C×40hr | Comp. Example |
| 16 | C | 806 | 55 | 630 | 550 | 710°C×40hr | Comp. Example |
| 17 | D | 794 | 115 | 670 | 590 | 720°C×40hr | Comp. Example |
| 18 | D | 719 | 95 | 610 | 580 | 680°C×40hr | Comp. Example |
| 19 | E | 752 | 130 | 590 | 550 | 710°C×40hr | Comp. Example |
| 20 | Z | 805 | 100 | 580 | 530 | 720°C×40hr | Comp. Example |

**Table 3**

| Steel No. | Ferrite grain diameter (µm) | Area ratio of ferrite grain with aspect ratio of 4.0 or more (%) | Bending properties after stretching | Remarks |
|---|---|---|---|---|
| 1 | 3.5 | 13.1 | ○ | Example of this invention |
| 2 | 3.2 | 8.8 | ○ | Example of this invention |
| 3 | 2.8 | 12.4 | ○ | Example of this invention |
| 4 | 2.6 | 9.2 | ○ | Example of this invention |
| 5 | 4.4 | 11.6 | ○ | Example of this invention |
| 6 | 3.3 | 7.5 | ○ | Example of this invention |
| 7 | 4.1 | 13.9 | ○ | Example of this invention |
| 8 | 3.7 | 8.7 | ○ | Example of this invention |
| 9 | 4.5 | 14.6 | ○ | Example of this invention |
| 10 | 3.1 | 9.2 | ○ | Example of this invention |
| 11 | 6.4 | 13.3 | Δ | Comp. Example |
| 12 | 6.2 | 14.4 | Δ | Comp. Example |
| 13 | 4.4 | 15.8 | × | Comp. Example |
| 14 | 5.6 | 14.1 | Δ | Comp. Example |
| 15 | 4.7 | 18.4 | × | Comp. Example |
| 16 | 5.9 | 14.6 | Δ | Comp. Example |
| 17 | 5.4 | 13.9 | Δ | Comp. Example |
| 18 | 5.5 | 14.2 | Δ | Comp. Example |
| 19 | 4.1 | 22.4 | × | Comp. Example |
| 20 | 4.0 | 13.5 | × | Comp. Example |

### EXAMPLE 2

A slab was formed by continuous casting of each of steel E shown in Table 1 and the following steels:
Steel F (C: 0.31%, Si: 0.18%, Mn: 0.68%, P: 0.012%, S: 0.0033%, Sol. Al: 0.005%, N: 0.0040%, Ar₃ transformation point: 785°C, Ac₁ transformation point: 737°C),
Steel G (C: 0.23%, Si: 0.18%, Mn: 0.76%, P: 0.016%, S: 0.0040%, Sol. Al: 0.008%, N: 0.0028%, Cr: 1.2%, Ar₃ transformation point: 785°C, Ac₁ transformation point: 759°C),
Steel H (C: 0.32%, Si: 1.2%, Mn: 1.5%, P: 0.025%, S: 0.010%, Sol. Al: 0.006%, N: 0.0070%, Ar₃ transformation point: 804°C, Ac₁ transformation point: 746°C),
Steel I (C: 0.35%, Si: 0.20%, Mn: 0.68%, P: 0.012%, S: 0.0038%, Sol. Al: 0.005%, N: 0.0033%, Mo: 0.17%, Cr: 0.98%, Ar₃ transformation point: 773°C, Ac₁ transformation point: 754°C).

Then the slabs were heated to 1230°C and hot-rolled and annealed under the conditions shown in Table 4 to produce steel sheet Nos. 21 to 37 having a thickness of 4.5 m. Annealing was performed in a nitriding atmosphere (N₂ atmosphere). The ferrite grain diameter and the aspect ratio and area ratio of the ferrite grains of each of the resultant hot-rolled steel sheets were measured by the same methods as in Example 1, and the bending property after stretching was evaluated as in Example 1. Also, as in Example 1, it was confirmed that carbides were spheroidized.

The Ar₃ transformation point and the Ac₁ transformation point of each of steels F to I were determined from the equations (1) and (2), and the Ar₃ transformation point and the Ac₁ transformation point of each of steels G and I containing Cr or Mo were determined using the above-described correction terms.

The results are shown in Table 5. Table 5 indicates that in steel sheet Nos. 21 to 27 produced under the constant conditions except the cooling rate, steel sheet Nos. 22 to 26 produced at the cooling rates within the range of the present invention have excellent bending property after stretching. It is also found that in steel sheet Nos. 23 to 26, the area ratio of ferrite grains with an aspect ratio of 4.0 or more can be controlled to 10% or less. It is further found that in steel sheet Nos. 28 to 33 produced at a constant cooling rate, steel sheet Nos. 30 to 33 produced at a cooling termination temperature and a coiling temperature both of which are within the ranges of the present invention have excellent bending properties after stretching. It is further found that in steel sheet No. 33 produced at a cooling termination temperature of 600°C or less and a coiling temperature of 550°C or less, the area ratio of ferrite grains with an aspect ratio of 4.0 or more can be controlled to 10% or less. In the examples of the present invention, it was confirmed that the average aspect ratio of carbides is 5.0% or less, and the carbides are spheroidized by spheroidizing annealing.

Steels E to I each having the composition within the range of the present invention, including steels G and I containing an ally element other than the basic components, exhibit excellent bending properties after stretching.

**Table 4**

| Steel sheet No. | Steel | Hot rolling condition | | | | Annealing of hot-rolled steel sheet | Remarks |
|---|---|---|---|---|---|---|---|
| | | Finishing temperature (°C) | Cooling rate (°C/sec) | Cooling termination temperature (°C) | Coiling temperature (°C) | | |
| 21 | F | 820 | 50 | 560 | 530 | 700°C×30hr | Comp. Example |
| 22 | F | 820 | 70 | 560 | 530 | 700°C×30hr | Example of this invention |
| 23 | F | 820 | 85 | 560 | 530 | 700°C×30hr | Example of this invention |
| 24 | F | 820 | 95 | 560 | 530 | 700°C×30hr | Example of this invention |
| 25 | F | 820 | 105 | 560 | 530 | 700°C×30hr | Example of this invention |
| 26 | F | 820 | 115 | 560 | 530 | 700°C×30hr | Example of this invention |
| 27 | F | 820 | 140 | 560 | 530 | 700°C×30hr | Comp. Example |
| 28 | F | 820 | 105 | 660 | 530 | 700°C×30hr | Comp. Example |
| 29 | F | 820 | 105 | 630 | 610 | 700°C×30hr | Comp. Example |
| 30 | F | 820 | 105 | 630 | 560 | 700°C×30hr | Example of this invention |
| 31 | F | 820 | 105 | 630 | 530 | 700°C×30hr | Example of this invention |
| 32 | F | 820 | 105 | 580 | 560 | 700°C×30hr | Example of this invention |
| 33 | F | 820 | 105 | 580 | 530 | 700°C×30hr | Example of this invention |
| 34 | E | 790 | 105 | 560 | 530 | 715°C×60hr | Example of this invention |
| 35 | G | 800 | 105 | 560 | 530 | 720°C×50hr | Example of this invention |
| 36 | H | 810 | 105 | 560 | 530 | 700°C×30hr | Example of this invention |
| 37 | I | 820 | 105 | 560 | 530 | 700°C×30hr | Example of this invention |

**Table 5**

| Steel No. | Ferrite grain diameter (µm) | Area ratio of ferrite grain with aspect ratio of 4.0 or more (%) | Bending property after stretching | Remarks |
|---|---|---|---|---|
| 21 | 5.4 | 13.2 | Δ | Comp. Example |
| 22 | 4.7 | 11.3 | ○ | Example of this invention |
| 23 | 3.6 | 8.8 | ○ | Example of this invention |
| 24 | 3.1 | 7.9 | ○ | Example of this invention |
| 25 | 2.9 | 8.5 | ○ | Example of this invention |
| 26 | 3.2 | 7.6 | ○ | Example of this invention |
| 27 | 4.5 | 21.9 | × | Comp. Example |
| 28 | 6.4 | 14.2 | Δ | Comp. Example |
| 29 | 5.8 | 14.6 | Δ | Comp. Example |
| 30 | 4.3 | 12.1 | ○ | Example of this invention |
| 31 | 4.0 | 13.3 | ○ | Example of this invention |
| 32 | 4.5 | 10.7 | ○ | Example of this invention |
| 33 | 3.9 | 8.4 | ○ | Example of this invention |
| 34 | 3.8 | 9.5 | ○ | Example of this invention |
| 35 | 3.7 | 8.7 | ○ | Example of this invention |
| 36 | 4.8 | 9.6 | ○ | Example of this invention |
| 37 | 3.5 | 8.8 | ○ | Example of this invention |

## Claims

1. A high-carbon hot-rolled steel sheet which is a hot-rolled spheroidized annealed material, the steel sheet comprising:
a composition consisting of, in % by mass, 0.2 to 0.7% of C, 2% or less of Si, 2% or less of Mn, 0.03% or less of P, 0.03% or less of S, 0.01% or less of Sol. Al, and 0.01% or less of N, optionally at least one selected from B, Cr, Ni, Mo, Cu, Ti, Nb, W, V, and Zr in the following content ranges in % by mass: B: 0.005% or less, Cr: 3.5% or less, Ni: 3.5% or less, Mo: 0.7% or less, Cu: 0.1% or less, Ti: 0.1% or less, Nb: 0.1% or less, W, V, Zr: 0.1% or less in total, the balance being Fe and inevitable impurities;
wherein a ferrite grain diameter is 5.0 µm or less, and an area ratio of ferrite grains with an aspect ratio of 4.0 or more is 15% or less;
wherein the ferrite grain diameter is an average grain diameter determined by approximating ferrite grains as circular grains in image analysis, and the aspect ratio is an average value of (major axis of ellipse)/(minor axis of ellipse) determined by approximating ferrite grains as elliptic grains in image analysis.

2. The high-carbon hot-rolled steel sheet according to claim 1, wherein the area ratio of ferrite grains with an aspect ratio of 4.0 or more is 10% or less.

## Patentansprüche

1. Kohlenstoffreiches heißgewalztes Stahlblech, das ein heißgewalztes weichgeglühtes Material ist, wobei das Stahlblech aufweist:
einen Zusammensetzung in Massen% bestehend aus:
0,2 bis 0,7 % an C,
2 % oder weniger an Si,
2 % oder weniger an Mn,
0,03 % oder weniger an P,
0,03 % oder weniger an S,
0,01 % oder weniger an Sol.Al, und
0,01 % oder weniger an N,
optional aus mindestens einem Bestandteil, das ausgewählt ist aus
B, Cr, Ni, Mo, Cu, Ti, Nb, W, V und Zr in den folgenden Anteilsbereichen in Massen%:
B: 0,005 % oder weniger,
Cr: 3,5 % oder weniger,
Ni: 3,5 % oder weniger,
Mo: 0,7 % oder weniger,
Cu: 0,1 % oder weniger,
Ti: 0,1 % oder weniger,
Nb: 0,1 % oder weniger,
W, V, Zr: insgesamt 0,1 % oder weniger,
wobei der Rest Fe und unvermeidbare Verunreinigungen sind;
wobei ein Ferritkorndurchmesser 5,0 µm oder weniger beträgt und ein Flächenverhältnis von Ferritkörnern, die ein Aspektverhältnis von 4,0 oder größer haben, 15 % oder weniger beträgt;
wobei der Ferritkorndurchmesser ein mittlerer Korndurchmesser ist, der durch Approximieren von Ferritkörnern als kreisförmige Körner in einer Bildanalyse ermittelt wird, und das Aspektverhältnis ein Mittelwert ist aus: (Hauptachse einer Ellipse)/(kleine Achse der Ellipse), der durch Approximieren von Ferritkörnern als elliptische Körner in einer Bildanalyse ermittelt wird.

2. Kohlenstoffreiches heißgewalztes Stahlblech nach Anspruch 1, wobei das Flächenverhältnis von Ferritkörnern, die ein Aspektverhältnis von 4,0 oder größer haben, 10 % oder weniger beträgt.

## Revendications

1. Tôle d'acier laminée à chaud à haute teneur en carbone qui est un matériau recuit sphéroïdisé laminé à chaud, la tôle d'acier comprenant :
une composition constituée, en % en masse, de 0,2 à 0,7 % de C, 2 % ou moins de Si, 2 % ou moins de Mn, 0,03 % ou moins de P, 0,03 % ou moins de S, 0,01 % ou moins d'Al sol. et 0,01 % ou moins de N, éventuellement d'au moins l'un choisi parmi B, Cr, Ni, Mo, Cu, Ti, Nb, W, V et Zr dans les plages de teneur suivantes, en % en masse : B : 0,005 % ou moins, Cr : 3,5 % ou moins, Ni : 3,5 % ou moins, Mo : 0,7 % ou moins, Cu : 0,1 % ou moins, Ti : 0,1 % ou moins, Nb : 0,1 % ou moins, W, V, Zr : 0,1 % ou moins au total, le reste étant du Fe et des impuretés inévitables ;
dans laquelle un diamètre des grains de ferrite est de 5,0 µm ou moins, et un rapport surfacique des grains de ferrite ayant un rapport d'aspect de 4,0 ou plus est de 15 % ou moins ;
dans laquelle le diamètre des grains de ferrite est un diamètre de grain moyen déterminé en considérant de manière approchée les grains de ferrite comme des grains circulaires dans une analyse d'image, et le rapport d'aspect est une valeur moyenne de (axe majeur de l'ellipse)/(axe mineur de l'ellipse) déterminée en considérant de manière approchée les grains de ferrite comme des grains elliptiques dans une analyse d'image.

2. Tôle d'acier laminée à chaud à haute teneur en carbone selon la revendication 1, dans laquelle le rapport surfacique des grains de ferrite ayant un rapport d'aspect de 4,0 ou plus est de 10 % ou moins.
